

Sept. 2, 1952

F. S. MARTIN

2,609,201

SILICONE ELASTOMETER GOLF BALL CORE

Filed June 26, 1947



INVENTOR.  
FRANK S. MARTIN  
BY  
Charles C. Millson  
ATTORNEY

## UNITED STATES PATENT OFFICE

2,609,201

## SILICONE ELASTOMER GOLF BALL CORE

Frank S. Martin, Cranston, R. I., assignor to  
United States Rubber Company, New York,  
N. Y., a corporation of New Jersey

Application June 26, 1947, Serial No. 757,145

3 Claims. (Cl. 273—62)

## 1

The present invention relates to a novel golf ball core capable of giving improved golf ball performance.

For many years golf balls have been provided with a core of rubber or other yielding material about which rubber thread was tightly wound to form the golf ball body, and over this body of thread was provided a molded balata cover.

For a number of years golf balls have been provided with a liquid center such as paste, 10 honey, oil or water confined within a rubber shell so that the center and shell form a core. One of the best golf balls now on the market is a liquid center ball in which the core of the ball contains a pellet formed of a spherical thin 15 plastic container filled with castor oil. This pellet or center is disposed within a relatively thick shell of vulcanized resilient rubber. The core thus formed has rubber thread wound tightly thereupon in a highly stretched condition to form the ball body, and this body is disposed in a balata cover as above described.

Experienced golfers desire the following properties in a ball: long flight, good feel on the club when the ball is hit, good click sound when the ball is hit and when it is dropped on a hard surface, long life without getting out of shape, and a cover that stands up well and has a good white color of pleasing appearance. The castor oil center ball above described when made of 30 high quality components possesses all of these properties to a substantial degree.

The present invention relates to a golf ball in which the liquid center of the core just described is replaced by a relatively new material 35 possessing plastic or doughy properties so that it can be worked between the fingers like putty, and when rolled into a ball will bounce to approximately the same degree as a good quality solid rubber ball. This strange material has 40 been given the name of "bouncing putty" and will be hereinafter described in greater detail.

Golf balls having a core containing a center formed of this so-called bouncing putty in place of the liquid center above described, but which are otherwise constructed like the liquid center balls are found to give excellent performance and to possess properties superior to other high grade golf balls now on the market. Experienced golfers are particularly pleased with the click of this new ball and also with the feel or property of the ball to get quickly off of the club.

The various features of a golf ball having a core constructed in accordance with the present invention will be further understood from the following description when read in connection with the accompanying drawing, wherein:

Fig. 1 shows the major portion of a golf ball constructed in accordance with the present invention in sections and a minor portion in side view; and

## 2

Fig. 2 illustrates the core alone of the ball of Fig. 1, the center of the core being shown in side view while the two halves of the shell are shown in section and in spaced relation to each other.

The core of the golf ball illustrated in the drawing is designated in its entirety by the numeral 10. This core comprises a center 11 formed of a compound containing sufficient bouncing putty to impart to the center pronounced bouncing properties and also putty-like plasticity. The center 11 is disposed within a relatively thick shell of vulcanized natural rubber, synthetic rubber, or resinous material having elastic properties. The two halves of the shell designated by 12 and 12' in Fig. 2 of the drawing should be vulcanized or cemented together when finished to firmly unite them about the center 11.

20 After the core 10 has been constructed as just described rubber thread is tightly wound about this core as heretofore to form a body 13 of the desired size. A cover 14 which may be formed of balata is then molded about the body in a well known manner, and the cover is painted and branded with the maker's name or mark as heretofore.

25 The size and weight of golf balls have become standardized and are followed carefully by golf ball manufacturers. The diameter of the finished ball should be 1.68 inches. The other dimensions of the ball may vary widely depending upon the type of ball to be made. A golf ball constructed in accordance with the present invention and having a center 11 about  $\frac{3}{8}$  of an inch in diameter and a core 10 about  $1\frac{1}{16}$  inches in diameter was found to perform in a very satisfactory manner. The body 13 of tightly wound rubber thread and cover 14 having a thickness of several hundredths of an inch were constructed as heretofore.

30 The so-called bouncing putty used in the center 11 is preferably the solid gel-like heat reaction product of a dimethyl silicone oil with a minor portion of a compound of boron such as 45 pyroboric acid, boric anhydride or boric acid. This material has a specific gravity of about 1.03. It also has pronounced cold flow properties in that a ball of this material will flow out into a thin disk in the course of hours. It does not flow appreciably under a rapid blow but will flow readily under the application of a low steady pressure; it is also stable throughout a very wide temperature range. This bouncing putty may be 50 used alone to form the center 11, or it may be used with pigments, fillers or plasticizers employed to increase its weight or to modify its plastic properties or for other reasons.

55 One important result secured by using plasticizers is that plasticizers reduce the tendency of the bouncing putty to shatter under a rapid

blow. Experience has shown that while bouncing putty bounces like vulcanized rubber it can be shattered by a sharp blow. I have found that such tendency to shatter can be reduced very materially by the use of plasticizers such as zinc soaps of fatty acids, and is reduced to some degree by the use of fillers.

The following table shows how plasticizers reduce the tendency of bouncing putty to shatter, the parts being by weight and B. P. stands for 10 bouncing putty.

Table I

| Composition                               | Treatment              | Test                       |    |
|-------------------------------------------|------------------------|----------------------------|----|
| 1. 100 parts B. P.                        | No milling or heating. | Shattered fairly easily.   |    |
| 2. 100 B. P.                              | Heated and milled.     | Do.                        |    |
| 3. 100 B. P. and 100 zinc oxide.          | do.                    | More difficult to shatter. | 5  |
| 4. 100 B. P. and 10 zinc stearate.        | do.                    | Do.                        | 10 |
| 5. 100 B. P. and 10 Laurex <sup>1</sup> . | do.                    | Do.                        |    |
| 6. Composition of Table II given below.   | do.                    | Do.                        |    |

<sup>1</sup> Laurex is a fatty acid activator and plasticizer and may be described as a zinc salt of a mixture of fatty acids in which lauric acid predominates.

The above compositions, except the first, as indicated were heated to melting during a ten minute interval, stirred and then milled on a rubber mill for ten minutes to complete the mixing. They were tested by striking a small pellet, approximately  $\frac{1}{4}$  inch in diameter, a hard rapid blow with a hammer. Compositions 1 and 2 shattered fairly easily. Compositions 3, 4, 5 and 6 were increasingly difficult to shatter in the order they are listed. One composition containing the above described bouncing putty which is found to produce a very satisfactory center is the following, the parts being by weight:

Table II

|                                         |        |
|-----------------------------------------|--------|
| Bouncing putty                          | 100.00 |
| Zinc oxide                              | 100.00 |
| Barytes                                 | 66.66  |
| Zinc soaps of fatty acids (plasticizer) | 5.00   |
| Rubber blue (coloring)                  | 3.33   |
|                                         | 274.99 |

Examples of the zinc soaps of fatty acids are:

1. zinc soaps of coconut oil fatty acids
2. zinc soap of lauric acid
3. zinc soap of stearic acid

Golf ball cores having a diameter of  $1\frac{1}{8}$  inches but different centers all about  $\frac{3}{8}$  of an inch in diameter were dropped from a height of 100 inches onto a hard surface to test their rebound properties at a temperature of 80° F., with the following result.

Table III

|                                                  | Rebound, inches |
|--------------------------------------------------|-----------------|
| Core having center of 100% bouncing putty        | 67.8            |
| Core having center of compound of above Table II | 65.5            |
| Core having oil capsule center                   | 62.0            |

It is not entirely clear why a golf ball having a center formed of bouncing putty but otherwise constructed as heretofore should perform in such a satisfactory manner but professional golfers playing golf balls constructed in ac-

cordance with the present invention and unaware of the fact that it was constructed differently from the balls they were familiar with have repeatedly commented upon the highly desirable properties of this ball, as to click, feel and flight. They have also compared its playing properties with the castor oil center ball above described and believe it to have properties superior thereto.

Having thus described my invention, what I claim and desire to protect by Letters Patent is:

1. A golf ball core adapted to have rubber thread wound tightly thereupon to form the golf ball body; said core comprising a center formed of a mixture of a solid gel-like heat reaction product of a dimethyl silicone oil with a minor portion of a compound of boron added thereto and having pronounced bouncing properties that are equal to those of good vulcanized elastic rubber and also having putty-like plasticity, said mixture also containing at least about 5% of zinc soap based on the weight of said solid gel-like heat reaction product to substantially increase the shatter-resistant properties of the center and containing an inorganic filler, and a shell of vulcanized rubber surrounding and confining the center.

2. A golf ball core adapted to have rubber thread wound tightly thereupon to form the golf ball body; said core comprising a center formed of a mixture of a solid gel-like heat reaction product of a dimethyl silicone oil with a minor portion of a compound of boron added thereto and having pronounced bouncing properties that are equal to those of good vulcanized elastic rubber and also having putty-like plasticity, said mixture also containing at least about 5% of zinc stearate based on the weight of said solid gel-like heat reaction product to substantially increase the shatter-resistant properties of the center and containing an inorganic filler, and a shell of vulcanized rubber surrounding and confining the center.

3. A golf ball core adapted to have rubber thread wound tightly thereupon to form the golf ball body; said core comprising a center formed of a mixture of a solid gel-like heat reaction product of a dimethyl silicone oil with a minor portion of a compound of boron added thereto and having pronounced bouncing properties that are equal to those of good vulcanized elastic rubber and also having putty-like plasticity, said mixture also containing at least about 5% of zinc laurate based on the weight of said solid gel-like heat reaction product to substantially increase the shatter-resistant properties of the center and containing an inorganic filler, and a shell of vulcanized rubber surrounding and confining the center.

FRANK S. MARTIN.

#### REFERENCES CITED

The following references are of record in the file of this patent:

#### UNITED STATES PATENTS

| Number    | Name    | Date          |
|-----------|---------|---------------|
| 1,945,062 | Miller  | Jan. 30, 1934 |
| 2,354,017 | Hazell  | July 18, 1944 |
| 2,360,090 | Wilhelm | Oct. 10, 1944 |
| 2,541,851 | Wright  | Feb. 13, 1951 |

#### OTHER REFERENCES

"The Amazing New Chemical Family," pages 86-88, Oct. 6, 1945, The Oil and Gas Journal.